

## UNITED STATES PATENT OFFICE.

GEORGE E. GAIL, OF DETROIT, MICHIGAN, ASSIGNOR OF ONE-HALF TO ALEX SEITZ, OF WAYNE COUNTY, MICHIGAN.

## COMPOUND TO SOLDER ALUMINUM.

No Drawing.

Application filed March 12, 1926. Serial No. 94,325.

The present invention relates to a soldering compound, and more particularly to an improved compound for use with aluminum, and a method of making the same.

An object of the present invention is to provide a solder, which may be used with virgin aluminum, and a compound which may be used either with or without a soldering iron.

10 Another object of the invention is to provide a compound which may be made on a commercial scale and which may be economically produced and easily handled in use.

Various other objects and advantages of 15 the compound and the method of producing the same will be brought out and understood from the following detailed description of the present preferred compound and the present method of making the same.

20 In order to illustrate the invention the following proportions and ingredients are used and treated and admixed in the following manner for producing approximately twenty-five pounds of virgin solder, the 25 latter being the base of the improved compound.

First, approximately nine and one-quarter pounds of zinc are melted, and for the purpose of closing the grain or pores of the

30 zinc, the same is poured into cold water effecting the quick chill of the molten metal, and this treatment imparts to the block tin a greater capacity to alloy with zinc, and produces a final compound or solder which

35 is of a very fine grain. The zinc is then remelted and to it is added approximately fifteen and one-quarter pounds of block tin, the block tin being added very slowly and the mass being continuously stirred during

40 such addition. About one-quarter of a pound of lead is then added very slowly to the mass while being stirred, and approximately one-quarter pound of phosphorous tin is added during the stirring, and the

45 mass is kept in agitation for approximately fifteen minutes longer to effect a thorough mixing and distribution of the tin and lead throughout the molten mass.

After the mass has been thoroughly stirred, a block of wood in the shape of a two inch 50 cube, or other suitable size and shape desired, is attached to a pole or rod and forced downwardly into the mass of metal and held at or near the bottom of the mass for approximately fifteen minutes. The block of 55 wood in the molten metal is to produce the boiling of the metal and to determine a thorough admixture of the various ingredients, because the molten metal will not adhere to the block of wood and the block 60 of wood will thus produce a scum at the top of the mass which may be readily skimmed off to remove the impurities. After the impurities rising to the top of the boiling mass have been removed, there is then added 65 about one-quarter ounce of pure beeswax, which serves as a flux as it readily works through the entire mass of metal and drives up to the surface all of the smaller particles of impurities that turn green. The use of 70 beeswax in the mixture is found to be important as other fluxes have failed to bring out these green colored impurities.

The metal is now ready to be poured off 75 into an iron chill or mold which should first be raised to a temperature of approximately 150 degrees.

It is found that this new solder may be used with virgin aluminum and that the product may be handled with or without a 80 soldering iron.

What is claimed is:—

1. The method of compounding an aluminum solder which consists in first melting approximately nine and a quarter pounds of zinc, pouring the molten mass of zinc into a chilling fluid to close the pores of the zinc, remelting the zinc, slowly adding thereto approximately fifteen and a quarter pounds of block tin, then separately adding slowly approximately one quarter pound each of lead and phosphorous tin, stirring the mass to thoroughly intermix said ingredients, then immersing and maintaining near the bottom of the mass a block of wood to effect the boiling of the mass, and finally adding 85 90 95

approximately one quarter ounce of pure beeswax to the mass for separating the impurities therefrom for removal at the surface of the boiling mass.

5 2. An aluminum solder comprising a compound of the following ingredients in substantially the proportions named: zinc, nine and one quarter pounds; block tin, fifteen

and one quarter pounds; lead and phosphorous tin, each one quarter pound; and pure <sup>10</sup> beeswax, one quarter ounce; the compound being characterized by boiling and removal of impurities therefrom.

In testimony whereof I affix my signature.

GEORGE E. GAIL.